

## 1

3,151,194

**PROCESS FOR THE MANUFACTURE OF SHAPED BODIES FROM VISCOSE, AND THE PRODUCTS THUS OBTAINED**

Albert Willem Jacob van Doorn and Adrianius Marius van de Ven, Arnhem, Netherlands, assignors to American Enka Corporation, Enka, N.C., a corporation of Delaware

No Drawing. Filed Sept. 1, 1961, Ser. No. 135,457  
13 Claims. (Cl. 264—191)

This invention relates to improvements in the production of shaped bodies of regenerated cellulose rayon from viscose. This invention also relates to an improved viscose spinning solution. More particularly, this invention relates to the production of films, fibers, threads, filaments and the like products from an improved viscose rayon spinning solution.

In conventional methods of producing shaped bodies from viscose, a suitable cellulosic material, such as wood pulp, is first converted into an alkali cellulose by treatment with a caustic soda solution. Thereafter, the treated cellulose is shredded and allowed to age. After ageing, the alkali cellulose is converted into cellulose xanthate by treatment with carbon disulfide. The cellulose xanthate is subsequently dissolved in a caustic soda solution in an amount sufficient to provide a viscose of the desired cellulose and alkali content. After infiltration, the viscose solution is allowed to ripen and is then extruded through a shaped orifice into a suitable coagulating and regenerating bath.

In the production of shaped bodies such as filaments, the viscose solution is conventionally extruded through a spinneret into a coagulating and regenerating bath consisting of an aqueous acid solution containing zinc sulfate. Thereafter, the filament is passed through a hot aqueous bath where it is stretched to improve its tensile strength. The filament may then be subjected to a dilute aqueous solution of sulfuric acid and sodium sulfate to complete the regeneration of the cellulose in the case where it is not completely regenerated upon leaving the stretching stage. The filament is subsequently subjected to washing, purification, bleaching, and drying treatments.

The threads and filaments formed by these conventional methods consist of a skin or outer shell portion and a core portion with a line of demarcation between the two. These threads and filaments will hereinafter be referred to as threads and filaments having a so-called skin structure.

In the conventional process for making tire cord, a number of threads, as obtained from a spinning operation, are combined and plied. In such processes, it is well known that a loss of strength will occur as a result of the plying operation. That is, the strength of the manufactured cord as well as the double loop strength, is lower than the sum of the strength values of the component threads. Such losses of strength due to the threads being processed into cord will hereinafter be referred to as cord losses.

Moreover, it is well known that by using polymers of epoxyalkanes having a certain composition and mean molecular weight, that is, polymers of epoxyethane having a mean molecular weight between 3,800 and 4,200, these cord losses may be reduced.

## 2

In accordance with the process of the present invention it has unexpectedly been found that threads can be produced with the occurrence of even smaller cord losses by the addition of a polythiodiglycol to the viscose before being spun in a sulphuric acid spinning bath containing at least 2% by weight zinc sulphate. In addition, this new process offers the advantage that the strength of the threads and the resistance to abrasion obtained is greater, and the swelling value lower, than the respective values for the threads obtained heretofore in the prior art processes. Moreover, the threads obtained according to this invention have the additional advantage over the poly-epoxyethane modified threads in that they have a higher resistance to heat. This property is of particular importance for tire cords. Furthermore, the above-mentioned higher strength of the threads can be obtained while using lower acid concentrations in the spinning bath.

It is therefore an object of this invention to provide a method for making regenerated cellulose viscose rayon threads, fibers, films, yarns, cords and the like products having improved physical properties by utilizing a novel combination of modifiers.

Another object is to provide a new viscose spinning solution.

It is still another object of the invention to provide a new viscose spinning solution containing novel modifiers.

A further object of this invention is to provide threads, filaments and cords from an improved viscose spinning solution.

Still another object of this invention is to provide tire cords having high double loop strength and high resistance to abrasion.

It is still a further object of this invention to provide fibers having an improved washing fastness.

Other objects will be apparent from the following detailed description.

In accordance with this invention, artificial threads, filaments, fibers, films and the like products are manufactured from a viscose solution containing at least one polythiodiglycol. These compounds containing ethereal oxygen and sulfur are first added to a viscose solution and then spun into a sulfuric acid spinning bath containing at least 2% by weight of zinc sulfate.

The term "polythiodiglycol" as employed herein in the specification and claims is intended to refer to the polymers formed by the condensation of thiodiglycols of the formula  $\text{HO}-\text{C}_n\text{H}_{2n}-\text{S}-\text{C}_n\text{H}_{2n}-\text{OH}$  alone or in the presence of similar glycols, wherein  $n$  is an integer 2, 3, or 4. The term "polythiodiglycol" is employed in the generic sense; when it is intended to refer to a polymer prepared from a specific thiodiglycol of the above formula, the resultant polymer is referred to as a  $\text{C}_n$ -polythiodiglycol to indicate whether  $n$  is 2, 3, or 4. The condensation suitably may be carried out in the presence of a dehydrating catalyst. A specific example of the polythiodiglycols used in the present invention is the  $\text{C}_2$ -polythiodiglycol prepared by condensing thiodiglycol at a temperature of about 50 to about 200° C. in the presence of a dehydrating catalyst like hydrochloric acid. This reaction may also take place in the presence of glycols.

A thiodiglycol polymer is preferred in which the number of ethereal oxygen and sulphur atoms are practically

equal and wherein the polymer has a mean molecular weight between about 700 and 1,250.

In accordance with this invention it is possible to combine polythiodiglycols prepared in the absence of glycols with polyglycols to obtain a mixture wherein the oxygen and sulphur content may be varied in a way which is comparable with the variation which may be obtained by copolymerization of thiodiglycol and glycols within the molecule.

The polyglycols may be homopolymers, copolymers or block polymers. An example of a block polymer is:



wherein  $b$  is equal to 30 and the sum of  $a$  plus  $c$  is equal to 85. Therefore, by combining such polythiodiglycols and polyglycols it is possible to obtain artificial products having improved swelling value, strength, and resistance to heat compared with the products obtained from viscoses employing only the polyglycols or the polythiodiglycols alone. A preferred form of the polyglycols is polyepoxyethane which has a mean molecular weight of about 3,000.

An example of a viscose to which a mixture of a polythiodiglycol and a polyglycol has been added is a viscose containing 0.1% by weight (calculated on the weight of the viscose) of polyethylene oxide with a mean molecular weight of 3,000 and 0.1% by weight of polythiodiglycol with a mean molecular weight of 1,200.

In addition to the polythiodiglycols being combined with polyglycols, they may also be combined with one or more amine compounds of the formula:



where  $\text{R}_1$  is an aliphatic chain with at least 8 carbon atoms,  $n$  is 2, 3 or 4,  $v+w$  is at least 2, and neither  $v$  nor  $w$  may be zero. The quaternary ammonium derivatives of these compounds may also be used when combined with polythiodiglycols the substituted amines are preferred in an amount ranging from about 25% to about 60% of the combined weights of the polythiodiglycols and the amines.

Examples of these amines are the products that are commercially available under the names Ethomeen C/15, Ethomeen C/20, Ethomeen C/25, Ethomeen C/60, Ethomeen S/15, Ethomeen S/20, Ethomeen S/25, Ethomeen S/60, Ethomeen 2/15, Ethomeen T/20, Ethomeen T/25, Ethomeen T/60 and Huls V 1011 T. Examples of the quaternary ammonium derivatives are the compounds that are available under the trade name Ethoquads.

The Ethomeens are prepared by reacting amines derived from higher fatty acids with ethylene oxide. In this way the C-Ethomeens are derived from coconut oil, the S-Ethomeens from soy-bean oil and the T-Ethomeens from tallow. The numbers 15, 20, 25 and 60 following the capital C's, S's and T's indicate, after a deduction by 10, the number of ethylene oxide molecules that have been reacted with one molecule of the amine.

Huls V 1011 T is a representative of the groups of compounds of the formula:



in which  $\text{R}$  represents an alkyl radical having 8 to 24 carbon atoms, the sum of  $x$  plus  $y$  is a value between 5 and 25, neither  $x$  nor  $y$  being equal to zero.

These amines, or the quaternary ammonium derivatives thereof, bring about a reduction in the cord losses. This seems to be due to the fact that these amines give the threads a greater surface smoothness. With the application of the polythiodiglycols alone, or with the application of a mixture of polythiodiglycols and polyglycols, a less smooth surface is obtained. A smooth surface attracts and retains less dirt and foreign matter. After

such smooth threads have been cut into staple, they are very suitable for use as carpet fibers. These staple fibers moreover, exhibit good wash fastness.

The polythiodiglycols, with or without the polyglycols or amines, may be added to the cellulose itself, or they may be added at any random stage in the preparation of the viscose. It is preferred that this addition be made after the cellulose xanthate has dissolved. These substances may, moreover, be added in concentrated form or after they have been dissolved in an alkali hydroxide or after they have been diluted with water. It is preferred that these modifiers be employed in an amount equal to about 0.03 to about 1.0% based on the weight of the viscose.

The composition of the viscose may vary within wide limits as far as the cellulose and alkali contents are concerned. It is preferred that the cellulose content be maintained between about 4 and about 8% by weight and the alkali content may also be maintained between the same limits.

Although spinning baths with a higher sulphuric acid content may be used, that is, baths containing up to 10% by weight or more of sulphuric acid, it has been found favorable, in connection with the desirable strength and water swelling properties of these threads to use spinning baths in which the sulphuric acid content is less than 7% by weight.

Preferably, the cellulose and alkali values are so chosen that the acid content of the spinning bath is less than 5.5% by weight and not higher than 1.2 times the alkali content of the viscose. The carbon disulphide content of the viscose is preferably chosen between about 26 and about 42% by weight, as calculated on the weight of the cellulose. It has also been found possible that the viscose modified according to this invention may be spun with an acid concentration that is below the acid concentration of the spinning bath.

In accordance with this invention, it is necessary that at least 2% by weight of zinc sulphate be employed. Above this minimum value of 2% by weight, the zinc content in the spinning baths may vary considerably and may be as much as 10% by weight or more. For reasons of economy, however, the lower percentages are preferred.

The stretching or drawing which is necessary for obtaining threads having the properties desired may be carried out in a single bath process as well as in a two bath process, that is, the stretching may be carried out in one or more stages. The length of the stretching zone in such a second bath of the two bath process is usually chosen such that at the end of the stretching process the cellulose xanthate is to a large extent decomposed, preferably to a cellulose xanthate ratio of not more than about 0.02. By the xanthate ratio, which is determined according to the method also known for the determination of the gamma number, is meant the ratio of the number of xanthate radicals still present to the total number of the glucose radicals ( $\text{C}_6\text{H}_{10}\text{O}_5$ ).

In accordance with this invention, it has been unexpectedly found when the viscose spinning solution contains a polythiodiglycol, a polyglycol and an amine, it has been found that the fibers, films, filaments, threads, cords and like products thus obtained exhibit greater tensile strength, lower cord losses, a greater abrasion resistance, lower swelling values, higher heat resistance, lower dirt retention, a smoother surface structure and greater wash fastness than the respective values for similar shaped bodies obtained according to prior art processes.

The invention will be further explained with reference to the following examples which are to be regarded by no means as restrictive. In these examples the composition of the viscose, the spinning bath, etc., is expressed in percentages by weight.

#### Example I

A viscose spinning solution was prepared with a cellulose content of 7.5%, an alkali content of 5.8% and 0.1%

of  $C_2$ -polythiodiglycol (calculated on the weight of the viscose) with a mean molecular weight of about 1,000. The solution, with a xanthate ratio of 0.43 and a viscosity of 80 seconds (determined by the falling sphere method), was spun into an aqueous spinning bath maintained at 55° C. This bath contained 5.3% of sulphuric acid, 11.0% of sodium sulphate and 5.0% of zinc sulphate. The thread was immersed for a distance of 100 cm. in this bath while passing through a tube consisting of two sections measuring 60 cm. and 20 cm. in length, respectively, and measuring 20 mm. and 40 mm., respectively, in diameter. The freshly spun thread was withdrawn from the spinning bath and was then stretched 50% in the atmosphere and was subsequently stretched 50% in a second bath containing 3.0%  $H_2SO_4$  and less than 1.0% of salts. The temperature of the second bath was 95% C. and the length of immersion in this bath was 120 cm. The thread was subsequently wound onto a bobbin at a speed of 40 meters per minute. The thread thus obtained was then washed free from acid in the usual manner, sized and then dried under tension. Thereafter, the physical properties were determined. The thread, which had a total tex (calculated as  $\frac{1}{6}$  of the denier) of 200 and consisted of 1000 filaments, was found to have a swelling value of 67%.

#### Example II

A viscose was prepared containing 5.5% by weight of cellulose, 5.5% by weight of sodium hydroxide, and containing 0.1% of polyethylene oxide with a mean molecular weight of 1,500 as well as 0.1% of  $C_2$ -polythiodiglycol with a mean molecular weight of 800. While at a xanthate ratio of 0.46 and a viscosity of 120 seconds (falling sphere method), the viscose was spun through a spinning nozzle having 1,200 holes, each measuring 60 microns in diameter, into a spinning bath maintained 50° C. This spinning bath contained 5.0% sulphuric acid, 15.0% sodium sulphate and 6.0% zinc sulphate.

The freshly spun threads passed through a tube as described in Example I and covered a distance of 100 cm. The threads were then withdrawn from the spinning bath and stretched 95% in a second bath maintained at 95° C. and containing 3.0% sulphuric acid. The length of immersion in this bath was 150 cm.

After the threads had been stretched they were collected at a rate of 40 meters per minute in a spinning pot and subsequently washed, subjected to an after treatment and dried in the usual manner. The threads thus manufactured had a swelling value of 63%.

These threads were then heated for 16 hours at 165° C. Thereafter it was noted that their strength had decreased to approximately 80% of the original value. On the other hand, threads obtained from viscose mixed exclusively with 0.2% of polyethylene oxide, were found to have a strength equal to only about 70% of the original value.

#### Example III

A viscose was prepared containing 7.5% by weight of cellulose, 5.8% by weight of sodium hydroxide, and containing 0.1% of  $C_2$ -polythiodiglycol with a mean molecular weight of 1,200, as well as 0.1% of the commercially available Ethomeen C/25. While at a xanthate ratio of 0.44 and a viscosity of 90 seconds (falling sphere method), this viscose was spun through a spinning nozzle having 1650 holes each measuring 50 microns in diameter, into a spinning bath maintained at 50° C. and containing 5.2% by weight of sulphuric acid, 14.0% sodium sulphate, 6.0% zinc sulphate and 0.005% lauryl pyridinium sulphate.

The freshly spun threads passed through a tube like that described in Example I and covered a distance of 100 cm. The threads were then withdrawn from the spinning bath and were stretched 95% in a second bath 120 cm. in length and containing 3.0% sulphuric acid. This bath was maintained at a temperature of 95° C.

After the threads had been stretched they were collected at a rate of 30 meters per minute in a spinning pot

and subsequently washed, subjected to an after-treatment and dried in the usual manner. The threads thus manufactured had a swelling value of 65%. When the threads were processed into cord, the cord loss was only 18%, as compared with 25% if no Ethomeen had been used in the viscose.

While preferred embodiments of the invention have been disclosed, the description is intended to be illustrative only and it is to be understood that changes and variations may be made without departing from the spirit and scope of the invention as defined by the appended claims.

What is claimed is:

1. A process for the manufacture of viscose rayon thread which comprises adding to a viscose solution a small amount of a polythiodiglycol selected from the group consisting of the polymers formed by the condensation of thioldiglycols of the formula



20 wherein  $n$  is an integer selected from the group consisting of 2, 3 and 4, and polymers formed by the condensation of said thioldiglycols in the presence of glycols corresponding thereto, and spinning the resultant viscose solution into a sulfuric acid coagulating bath containing at least 2.0% by weight of zinc sulfate to form smooth threads, said small amount of said polythiodiglycol being effective to provide threads having improved strength, abrasion and heat resistance, lower swelling value and when twisted into cord has lower cording losses.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560

10. A process according to claim 1 wherein preliminary to said spinning step from about 0.03 to about 1.0% by weight, based on said viscose, of a polyethylene oxide also is added to said viscose solution.

11. A process according to claim 10 wherein the amount of said polythiodiglycol employed is in the range of from about 0.03 to about 1.0% by weight based on said viscose, and said polyethylene oxide has a mean molecular weight in the range of from about 1,500 to about 10 3,000.

12. A process according to claim 11 wherein said polythiodiglycol has a mean molecular weight in the range of from about 700 to about 1,250.

13. A process according to claim 12 wherein said polythiodiglycol is a homopolymer of



**References Cited in the file of this patent**

**UNITED STATES PATENTS**

|           |                        |                |
|-----------|------------------------|----------------|
| 2,392,103 | Schlosser et al. ----- | Jan. 1, 1946   |
| 2,393,817 | Schlosser et al. ----- | Jan. 29, 1946  |
| 2,696,423 | Dietrich -----         | Dec. 7, 1954   |
| 2,852,333 | Cox et al. -----       | Sept. 16, 1958 |
| 2,912,299 | Drisch et al. -----    | Nov. 10, 1959  |
| 2,962,341 | Cox -----              | Nov. 29, 1960  |
| 2,983,572 | Elling et al. -----    | May 9, 1961    |